

## UNITED STATES PATENT OFFICE.

CARMELO BIONDO, OF BOSTON, MASSACHUSETTS.

## WATERPROOFING CLOTH.

No Drawing.

Application filed February 12, 1921. Serial No. 444,599.

*To all whom it may concern:*

Be it known that I, CARMELO BIONDO, a subject of the King of Italy, and resident of Boston, county of Suffolk, Commonwealth 5 of Massachusetts, have invented an Improvement in Waterproofing Cloth, of which the following description is a specification.

This invention relates to the waterproofing of cloth, such as articles of wearing apparel 10 and while applicable to other kinds of fabric is well adapted and designed for waterproofing woolen cloths. A principal object of the invention is to provide means for rendering a cloth of wool or other material 15 substantially waterproof, while still retaining its original porous and pliable condition in large degree. A further object is to provide for waterproofing a fabric in a manner so that its appearance and qualities in use 20 are not materially affected. To this end the invention consists in an improved formula for a waterproofing solution into which the cloth is dipped, and in an improved method of treating the cloth in connection with this 25 solution.

In preparing the waterproofing solution of my invention, I heat to the boiling point ten liters, i. e., a little more than two gallons of water. To this is first added one pound 30 of sodium carbonate which is dissolved therein by stirring. I then add one ounce of castor oil and one ounce of spirits of turpentine. I then stir into the hot solution two pounds of alum. This results in a 35 chemical reaction wherein the mass increases about four times in volume and becomes of a foamy and milky consistency. The action of the alum upon the solution is to convert it partially into a resinate and oleate of 40 aluminum. The stirring of the solution is continued until it becomes again thin and fluid. It is then drawn into a wooden receptacle and again stirred a short while 45 after which it is allowed to set about twenty hours. The solution is then again placed in a metal vessel and heated to about forty degrees C. Then the cloth to be treated is dipped into the solution and left about two

hours,—i. e., until the water is cooled. The cloth is then rinsed to a fair degree,—but 50 not too much and allowed to dry. When thoroughly dry it is immersed and rubbed in clean water three or four times, the water being changed each time. This is done until the cloth becomes again soft and pliable, and 55 after being allowed to dry it is ready for use. In the practice of the invention certain equivalents may be used to some extent in place of those named; thus in place of the turpentine, alcohol with a variety of rosin 60 known as "Greek tar" may be employed, and for the castor oil olive oil and cocoa oil may be substituted. I therefore desire the benefit of a reasonable range of equivalents with respect to the appended claims. 65

Having described my invention, what I claim as new and desire to secure by Letters Patent is:

1. The herein described method of making a waterproofing solution which consists 70 in adding to ten liters of hot water, one pound of sodium carbonate and one ounce of castor oil, one ounce of spirits of turpentine and then stirring in two pounds of alum. 2. A waterproofing solution made up of 75 the reaction products of approximately ten liters of water, one pound of sodium carbonate, one ounce of castor oil, one ounce of spirits of turpentine and two pounds of alum. 80

3. The herein described method which consists in providing a waterproofing solution containing resinate and oleate of aluminum, dipping the fabric to be treated therein for a substantial interval, drying and 85 then washing the fabric.

4. The herein described method which consists in providing a waterproofing solution as set forth in claim 1, immersing the fabric to be treated therein for a substantial interval, partially rinsing the fabric, drying the same, and then cleansing the fabric with 90 water.

In testimony whereof, I have signed my name to this specification.

CARMELO BIONDO.